

Dec. 15, 1959

W. BOYER ET AL

2,916,910

STEEL REINFORCEMENT FOR REINFORCED CONCRETE STRUCTURES

Filed March 14, 1957



INVENTORS  
WILHELM BOYER  
KUNO EISENBURGER  
WALTER HUFNAGL  
JOSEF RITTER  
BY

ATTORNEY

# United States Patent Office

2,916,910

Patented Dec. 15, 1959

1

2,916,910

## STEEL REINFORCEMENT FOR REINFORCED CONCRETE STRUCTURES

Wilhelm Boyer, Graz, and Kuno Eisenburger, Wels, Austria, Walter Hufnagl, Munich, Germany, and Josef Ritter, Graz, Austria, assignors to EVG Entwicklungs- und Verwertungsgesellschaft m.b.H., Graz, Styria, Austria

Application March 14, 1957, Serial No. 645,977

9 Claims. (Cl. 72—110)

The invention relates to steel reinforcements for reinforced concrete structures, and has the main object of providing steel reinforcements which combine high permissible steel stresses with high adhesive strength between the steel reinforcements and the concrete.

This is a continuation-in-part of our application Serial No. 344,082, filed March 23, 1953, and now abandoned.

The development of reinforcing rods for reinforced concrete is based on the desire to apply higher stresses to the steel in the reinforcement and thus to reduce the total amount of steel in the concrete. Calculations of the stresses on the rods are valid only if the forces which correspond to the increased stresses in the steel can be transmitted from the steel to the concrete or vice versa by an improved adherence or another anchorage of the reinforcing rods in the concrete.

The earliest and simplest form of a reinforcing rod for reinforced concrete is a round rod having a relatively smooth surface. When such a round or sectional rod is used as a reinforcement in concrete, a tensile load will cause a transverse contraction of the rod, which results in loosening the reinforcement in the concrete; the remaining bond between the concrete and steel is sufficient for steel stresses up to a maximum of 20,000 pounds per square inch (p.s.i.) but is not sufficient if a substantial additional increase of the permissible stress in the steel is desired in accordance with the invention.

Various other special designs of reinforcing elements have been proposed to improve the anchorage of the reinforcing bars in the concrete. For instance, round rods having helically twisted longitudinal ribs thereon, and pairs of rods which have been twisted together have been suggested. Whereas in both cases a better anchorage is achieved than with round rods and enables the permissible steel stress to be increased to about 28,000 p.s.i., the anchorage forces are transmitted only by the roughness of the surface and by the resistance to rotation at the helically twisted contact surface of the reinforcements. Thus oblique components of force are set up in the concrete, which can produce wedge effects resulting in an unfavorable stress pattern in the concrete.

According to another proposal, a reinforcing rod having grooves in its sides is formed with transverse ribs in the grooves which form anchoring surfaces extending at right angles to the rod axis. Whereas this provides for a good anchorage in the concrete, which permits also of steel stresses up to 28,000 p.s.i., a further increase of the permissible steel stresses is not possible without difficulty because, in such reinforcing rods, an unfavorable ratio between the steel cross-section to the anchoring rib surface area is obtained. For various reasons that ratio can hardly be improved. This is so because an increase in the rib surface area would involve the danger of a local reduction in quality at the position of the ribs if the reinforcing elements are made of high-grade steel, and because more highly protruding ribs would not only be subjected to high bending stresses but would also render the manipulation and storage of such reinforcing

2

elements more difficult. Finally, such reinforcing elements can be made only by hot-pressing or hot-rolling and can, therefore, be given a high yield point only by correspondingly large amounts of alloying constituents, involving high cost.

It is an object of the invention to provide a novel reinforcing element which ensures a perfectly safe anchorage in the concrete and a reliable transmission of forces between the concrete and steel even if the adherence with the concrete is loosened by a transverse contraction under tensile stress, and which involves no difficulties in handling and can be manufactured with ease, particularly in a high-grade condition, i.e., with a high yield point, by cold drawing at low cost.

It is another object of the invention to provide welded steel reinforcements which combine a high yield point with good welding properties.

It is a further object of the invention to provide strip shaped reinforcement steels which allow comparatively easy shaping by bending out of the plane of the strip while being comparatively stiff in the plane thereof.

It is yet another object of the invention to provide reinforcement grid systems which combine the characteristics of the individual reinforcements referred to hereinabove.

With these and other objects in view we provide a reinforcement steel strip for reinforced concrete structures comprising in combination: longitudinal rods consisting of steel of a comparatively high yield point arranged parallel to one another, and transverse connectors inter-

welded with the said longitudinal rods at intervals. For example the longitudinal rods may consist of a steel having a yield point of more than 70,000 p.s.i. and of a higher content in carbon and/or manganese than the transverse connectors. The distance between parallel longitudinal rods is of the same order of magnitude as their own thickness, about equal for rods of 0.8 inch thickness or more, but not less than 0.8 inch for thinner rods. A spacing of about 0.8 inch and 1.2 inches is suitable in most instances. The interval between the transverse connectors is usually of a higher order of magnitude than the distance between the longitudinal rods, and does not exceed 8 inches.

The transverse connectors may be pieces of rods or of plates, the latter may be put edgewise across the longitudinal direction of the longitudinal rods with their flat faces extending at right angles to the longitudinal rods.

When such a reinforcing element is embedded in concrete the latter will penetrate into the spaces between the longitudinal rods and will form between the adjacent transverse webs thick bridges on which the transverse webs are supported. The flat faces of the transverse webs or connectors prevent a transmission of detrimental oblique forces to the concrete. Then the reinforcing element is subjected to tensile stress only the adherence between the contacting concrete and steel surfaces can be eliminated whereas the anchorage formed by the transverse webs and concrete bridges will remain intact. That anchorage is so strong that any holding head previously required at the ends of the reinforcing element and provided mostly by the bending of end hooks can be omitted.

As will be explained hereinafter the ratio of the spacing between the transverse connectors or webs to the spacing between the longitudinal rods must be less than

2.4

$\phi$

where  $\phi$  is the diameter of the longitudinal rods in inches, in order to make certain that the width of the cracks forming in the concrete does not exceed the permissible maximum value of  $1/100$  inch. The optimum value for the spacing between the webs depends on the concrete quality, on the permissible steel stress and on the diam-

eter of the longitudinal rods. If a value smaller than the optimum is chosen a larger amount of steel is required but the reinforced concrete is not adversely affected thereby. The thickness of the transverse webs should be in the range from 0.4-0.75 inch.

In order to achieve a perfect welded joint between the longitudinal rods and transverse webs or connectors the latter should be made of a softer steel than the former. The longitudinal rods may be worked by cold drawing or their high yield point may be due to an appropriately high content of alloying constituents such as C and/or Mn. The transverse webs should not contain more than a relatively small content of said elements.

It has been found that reinforcement strips and grids according to the invention allow the use of a steel of a yield point of about 4000 kilograms per square centimeter and of correspondingly high permissible tensile stresses, and at the same time give such an improved adhesive strength between the steel reinforcements and the concrete that the unavoidable cracks in the concrete do not exceed 0.15 to 0.20 millimeter in width whereby the danger of dampness or vapors penetrating right to the steel reinforcements and causing corrosion is greatly reduced and the durability of the reinforced steel construction is improved. Owing to better adhesion of the concrete to the steel reinforcements the distances between adjacent cracks are also reduced. The width of the cracks measured on concrete structures using the reinforcement steel according to the invention has proved to be in good agreement with calculated values. For example, with a steel of a permissible tensile stress of 3000 kilograms per square centimeter and a modulus of elasticity of 2,100,000 kilograms per square centimeter and a distance 100 millimeters between transverse connectors the calculated width of cracks is

$$\frac{3000 \times 100}{2,100,000} = 0.14 \text{ millimeter}$$

Conversely the required interval between transverse connectors can be calculated on the basis of the permissible width of cracks, on the basis of the permissible tensile stress and modulus of elasticity of the steel used for the longitudinal members of the reinforcement strips according to the invention.

For a better understanding of the invention, reference may be had to the accompanying drawings in which:

Figure 1 of the drawing is a perspective view of a reinforcing element embodying the present invention;

Figures 2 and 3 respectively are a top plan view and a cross-sectional view of a reinforcing element;

Figure 4 is a schematic illustration in perspective of a test set up for determining the reinforcing strength and the required dimensions of the reinforcing elements according to the invention;

Figure 5 is a cross-section view of the reinforcing element illustrating dimensions on which tests are based;

Figure 6 is a cross-section view of a concrete beam reinforced with a reinforcing element of the kind shown in Figures 1 and 5;

Figure 7 is a side elevational view of the concrete beam supported at its ends and under load; and

Figure 8 and Figures 8a, 8b, 8c, and 8d illustrate schematically the stresses on the concrete beam when a crack occurs in the beam.

The reinforcement steel according to Figures 1 to 3 has a strip-like shape and consists of two longitudinal rods 11a and 11b which are parallel and are connected with one another by pieces of rod 12 or other web forming material lying between them and interwelded with the longitudinal rods. The transverse webs 12 are spaced from one another lengthwise of the rods 11a, 11b a distance s. The longitudinal rods 11a, 11b in particular consist of a steel having a high yield point. The cross-section of the longitudinal rods 11a, 11b may be round, or profiled, as the case may be; the cross-section of the

transverse webs 12 may be oval, square or oblong, such oblong cross-section profiles being positioned on edge relative to the longitudinal dimension of the reinforcement strip, if desired. Thus each transverse web may consist of a separate form piece produced e.g., by pressing, stamping or the like.

The interwelded transverse webs 12 form an absolutely rigid connection between the two longitudinal rods 11a, 11b which completely prevents any sliding of the reinforcement relative to the concrete in the zone of the webs; the anchor resistance can be overcome only by complete destruction of the tension zone of the concrete. By controlling the spacing between the transverse web 12 the permissible width of cracks can be determined, assuming an appropriate quality of the steel. The spacing between the transverse webs should be less than 200 millimeters (8 inches).

As regards the spacing a between the two longitudinal rods 11a and 11b, it should be equal to the diameter or thickness of the rods; with a rod diameter below 20 millimeters the clearance spacing should not be less than 20 millimeters (0.8 inch). When two longitudinal rods 11a, 11b interconnected by one or more interwelded transverse webs 12 are embedded in a concrete cube 13, as is shown in Figure 4, and the protruding longitudinal rods are subjected to tension in the sense of the arrow P, the first slight movement of the reinforcing element will occur with any concrete quality and independently of the diameter  $\phi$  of the longitudinal rod when the calculated average pressure of the concrete on the transverse web 12 exceeds the value

$$2f'_c \quad (1)$$

where  $f'_c$  is the ultimate compressive strength of concrete. Said movement can be observed with a dial gauge 14.

When the average pressure of the concrete on the transverse web exceeds the value

$$12f'_c \quad (2)$$

the concrete will be destroyed and the longitudinal rods as well as the transverse web will be pulled out of the concrete.

To confirm the dimensions specified for the reinforcing elements according to the invention the cross-section of a reinforcing element according to the invention as shown in Figure 5 will be considered first. The diameter of the longitudinal rods 11a, 11b is designated  $\phi$ , the spacing between said rods is designated a. The dimension a is at the same time a sufficiently accurate specification of the length of the transverse webs 12, which are interwelded to the longitudinal rods 11a, 11b. On the one hand the width of the transverse webs should be as large as possible to ensure that the transverse web provides the largest possible anchoring surface area for reinforcing element; on the other hand the height of the transverse webs should not exceed the diameter  $\phi$  of the longitudinal rods so that the transverse webs do not protrude over the longitudinal rods, which would render the handling and storage of the reinforcing elements according to the invention more difficult. For this reason the width of the web is made to equal the diameter  $\phi$  of the longitudinal rods. Thus the cross-sectional area or effective area  $F_s$  presented by the web to the concrete equals

$$F_s \approx a\phi \quad (3)$$

The entire steel cross-section  $A_s$  of the two longitudinal rods is

$$A_s = \phi^2 \frac{\pi}{2} \quad (4)$$

Therefore:

$$\frac{F_s}{A_s} = \frac{2a}{\phi\pi} \quad (5)$$

In the ensuing explanation, and as used elsewhere

throughout this application, the values  $f_c$ ,  $f'_c$ ,  $f_{ct}$  and  $f'_{ct}$  have the following meaning:

- $f_c$ —compressive stress of concrete  
 $f'_c$ —ultimate compressive strength of concrete  
 $f_{ct}$ —tensile stress of concrete  
 $f'_{ct}$ —ultimate tensile strength of concrete

Figures 6 and 7, respectively, are a cross-sectional view and a side elevation showing a rectangular concrete beam having the width  $b$  and the height  $d$  and reinforced in the tension zone with a reinforcing element according to the invention. As is apparent from Figure 7 that beam is supported at its ends and loaded. An increase in the load on the beam will cause a crack to form in the tension zone, e.g., at the point  $x$ , because the tensile stress  $f_{ct}$  has exceeded the ultimate tensile strength  $f'_{ct}$  of concrete. At that point  $x$  the reinforcement must take up the entire tensile stress because the locally cracked concrete can no longer take up any stress. At the point  $y$ , spaced by the distance  $e$  from the point  $x$  no crack has been formed at that time and high tensile stresses are effective in the concrete so that the reinforcement is subjected only to little stress. In that condition, therefore, the stress distributions  $f_c$  and  $f_{ct}$ , respectively, shown below Figure 7 (in Figure 8c for the cracking position  $x$ , in Figure 8d for the undamaged position  $y$ ) are obtained. The stresses actually taken up by the concrete are shown as hatched areas, while the tensile stress taken up by the reinforcement is shown as a clear area. If the tensile stresses  $f_{ct}$  in the concrete exceed the ultimate tensile strength  $f'_{ct}$  also at the point  $y$  a second crack will be formed and the stress distribution shown in Figure 8c in Figure 7 below point  $x$  will be obtained also at point  $y$  as shown in Figure 8d.

If several transverse webs 12 of the reinforcing element according to the invention are disposed between the first cracking point  $x$  and the point  $y$  considered, a stepped stress distribution  $f_s$  and  $f_{ct}$  according to Figures 8a and 8b will be obtained in the longitudinal rods and in the concrete before a crack occurs at  $y$ . The stepwise stress reduction in the longitudinal rods corresponds to the stepwise increase of the tensile stresses in the concrete. The stress steps are disposed at the positions of the transverse webs, which absorb the stress step with their effective web surface areas  $F_s$ . Regarding the test results explained with reference to Figure 8 a transverse web having an effective area  $F_s$  can transmit the force

$$F_s 2 f'_c \quad (6)$$

without moving in the concrete.

If the spacing of the transverse webs is designated  $s$ , the number of transverse webs in the distance  $e$  equals

$$\frac{e}{s}$$

The total force which can be transmitted by the transverse webs in the distance  $e$  without causing a movement of the reinforcement is, therefore,

$$\frac{e}{s} F_s 2 f'_c \quad (7)$$

On the other hand it is apparent from the diagram shown in Figures 8, 8c and 8d that the force required to set up the stress  $f'_{ct}$  in the outermost fiber in tension in the tension zone of the beam is determined by

$$\frac{bd}{2} (1-k) f'_{ct} \quad (8)$$

The factor,  $d(1-k)$ , as is well known, designates the distance of the neutral fiber from the tensioned edge (see Figure 8).

A second crack will be formed if the force introduced by the reinforcing element in the concrete according to Equation 7 corresponds to the force required to set up

the stress  $f'_{ct}$  in the outermost fiber in tension according to Equation 8.

It is usual to express the entire steel cross-section in a beam in relation to the concrete cross-section. This ratio  $p$  of tensile reinforcement is directly obtained from Figure 6 as

$$p = \frac{A_s}{bd}$$

10 or, with (5)

$$p = \frac{F_s \phi \pi}{2abd} \quad (9)$$

(If the beam is reinforced with several reinforcing elements,  $A_s$  is to be replaced by  $\Sigma A_s$  and  $F_s$  by  $\Sigma F_s$ .)

If it is further considered that the ratio  $f'_{ct}/f'_c$  amounts for several concrete qualities, on an average, to

$$f'_{ct} = \frac{1}{12} f'_c \quad (10)$$

20 then the equalization of the Expressions 7 and 8 and the substitution of (9), (10) and solution for  $s$  leads to the equation

$$s = \frac{96epa}{\pi \phi (1-k)} \quad (11)$$

In order to obtain an interpretable relation between the parameters  $s$ ,  $a$  and  $\phi$  of the reinforcing element the values  $e$ ,  $k$  and  $p$  must be determined.

The determination of the distance  $e$  between cracks is based on the rule that cracks in the tension zone of a reinforced concrete structure must not exceed a width of  $\frac{1}{100}$  inch but are permissible up to that harmless width. Because the concrete remains stressless in the tension zone between two cracks the width of the crack depends on the elongation of the reinforcing element on the distance  $e$  between the two cracks. If the steel stress is designated with  $f_s$  and the modulus of elasticity is designated with  $E_s$  an elongation of the reinforcing element by  $\frac{1}{100}$  inch will be obtained at

$$e = \frac{1}{100} \frac{E_s}{f_s} \quad (12)$$

If  $E_s = 30.10^6$  p.s.i. then

$$e = 3.10^5 \frac{1}{f_s} \quad (13)$$

For the determination of the value  $k$  the extreme cases of concrete quality in reinforced concrete structures may be considered, i.e., the lowest quality  $f'_c \text{ min.} = 1800$  p.s.i. together with the standarized permissible concrete stress  $f'_c \text{ min.} = 800$  p.s.i., and the highest concrete quality at present achievable,  $f'_c \text{ max.} = 6500$  p.s.i. and  $f'_c \text{ max.} = 3000$  p.s.i.

The value  $k$  is calculated according to the known formula

$$k = \frac{f'_c}{f_s + f'_c} \frac{n}{n} \quad (14)$$

60 wherein

$$n = \frac{E_s}{E_c}$$

65 equals the relation between the moduli of elasticity of steel and concrete; for the poorest concrete considered holds  $n = 15$ , for the best concrete  $n$  may be considered as equalling 6.

If the stated values of  $f_c$  and  $n$  are substituted in (14) and the steel stress is assumed according to the invention at its lower limit  $f_s = 35,000$  p.s.i. but at its upper limit in conjunction with the highest concrete quality as  $f_s = 50,000$  p.s.i., a mean  $k$  value of

$$k \sim 0.3 \text{ or } 1-k \sim 0.7 \quad (15)$$

70 75 can be computed for these two extreme cases.

A reinforced concrete beam is correctly reinforced if the tensile force  $T$  in the reinforcement is as great as the highest permissible compressive force  $C$  in the concrete.

The tensile force in the reinforcement equals

$$T = f_s A_s \text{ or, with (9), } T = f_s b d p \quad (16)$$

According to Figure 8 the compressive force in the concrete equals

$$C = f_c \frac{bkd}{2} \quad (17)$$

For  $C = T$

$$p = \frac{f_c k}{2f_s} \quad (18)$$

If the values derived according to (13), (15) and (18) for  $e$ ,  $k$  and  $p$  are substituted in Equation (11) then

$$s = 2.10^6 \frac{a f_c}{\phi f_s^2} \quad (19)$$

Thus the side ratio

$$\frac{a}{s}$$

of the rectangle included by the longitudinal rods 11a, 11b and two adjacent transverse webs 12 depends on the diameter  $\phi$  of the longitudinal rods and on the permitted stresses  $f_s$  and  $f_c$  in the steel and concrete. If the assumed extreme values  $f_c \text{ min.} = 800 \text{ p.s.i.}$  and  $f_c \text{ max.} = 3000 \text{ p.s.i.}$  are substituted in (19)

$$\frac{0.16 \cdot 10^{10}}{\phi f_s^2} \leq \frac{s}{a} \leq \frac{0.6 \cdot 10^{10}}{\phi f_s^2} \quad (20)$$

and, for  $\phi = \frac{1}{2}$  inch:

$$\frac{0.32 \cdot 10^{10}}{f_s^2} \leq \frac{s}{a} \leq \frac{1.2 \cdot 10^{10}}{f_s^2} \quad (21)$$

Furthermore, if the limits of

$$\frac{f_c}{f_s^2}$$

are calculated for the poorest and best concrete and steel qualities assumed, (19) gives with a small margin of tolerance

$$\frac{1.3}{\phi} < \frac{s}{a} < \frac{2.4}{\phi} \quad (22)$$

The lower limit for

$$\frac{s}{a}$$

applies to relatively poor qualities of the materials, the upper limit for the best qualities.

The spacing  $a$  of the longitudinal rods should be small to enable the reinforcing element according to the invention to be handled like a rod-shaped reinforcing element according to Figures 1 to 4. According to United States Standards it must not be less than 1 inch to ensure a safe penetration even of coarse concrete into the space between the longitudinal rods.

For the dimension  $a = 1$  inch, Equation 22 shows that

$$\frac{1}{\phi} < \frac{s}{a} < \frac{1.9}{\phi} \quad (23)$$

Thus the spacing of the transverse webs for  $\phi = \frac{1}{2}$  inch should be between 2.6 inches and 4.8 inches, depending on the concrete quality. In this connection, care is to be taken above all to remain below the upper limit of 8 inches for  $s$  because the width of cracks in the concrete would be increased if that limit is exceeded. A value below the lower limit is not critical because it will lead only to a somewhat increased consumption of web ma-

terial but has no detrimental consequences for the reinforced concrete structure.

The thickness  $i$  of the transverse webs should be such that the section modulus of said webs at the welded joint should be capable of absorbing the fixed-end moment of the transverse webs, which are considered beams gripped between the longitudinal rods, at the load obtained under the calculated stress condition, taking into account the yield point of about 30,000 p.s.i. of the steel used for the web. Since the static consideration of this problem involves great difficulty the tolerances for the thickness of the web have been determined experimentally. It was found that the thickness  $i$  of the web should meet the relation

$$0.4\phi < i < 0.75\phi \quad (24)$$

Compared to known reinforcements for concrete the reinforcing element according to the invention enables a reduction of steel in the range of 40-65%, with much reduced transport and handling costs.

The derivation of Formula 19 has been based on the assumption that the tensile force in the reinforcement of the reinforced concrete beam is to equal the maximum permissible tensile strength in the concrete. That requirement is not always fulfilled. There are many cases where the concrete is not loaded to its full carrying capacity. Owing to the underload on the concrete a smaller steel cross-section is required in such cases. Also in that case, however, the reinforcement should be designed so that the permissible width of crack will not be exceeded.

In order to observe the permissible width of crack on which Formula 16 is based even under the changed load and reinforcement conditions the total of the effective web areas, represented as the product of the individual web areas and the number of webs on a predetermined distance must be the same as under the optimum load conditions. This can be achieved by providing a graded series of reinforcing elements according to the invention, having different longitudinal rod diameters, and designing the distance of transverse webs in that specimen of the series which has the greatest longitudinal rod diameter according to Formula 16; that specimen is used for fully utilized concrete; the reinforcing elements of the series having longitudinal rods smaller in diameter have the same spacing of the transverse webs as the stronger reinforcing element designed according to Formula 16 and are used in less highly loaded concrete.

Equations 7 and 8 state that a certain web area  $F_s$  is required to obtain a width of crack not exceeding to  $\frac{1}{100}$  inch. A reduction of the steel cross-section involves also a reduction in the web area whereas Equation 5 shows the ratio

$$\frac{F_s}{A_s}$$

to increase with a decrease in the longitudinal rod diameter. This enables the total web area required to be ensured by maintaining the web spacing  $s$  constant when the longitudinal rod diameter is decreased.

If the concrete cross-section is fully utilized a longitudinal rod diameter of  $\phi = \frac{1}{2}$  inch, e.g., involves a required transverse web area  $F_s$  to produce a crack not exceeding  $\frac{1}{100}$  inch in width. If the concrete cross-section is utilized only by half so that only half the steel cross-section is required the use of two reinforcing elements having a longitudinal rod diameter of  $\frac{1}{4}$  inch will reduce the steel cross-section by half whereas the total transverse web area required according to Formula 5 for a web spacing calculated according to Equation 19 for  $\phi = \frac{1}{2}$  is retained.

The new reinforcement steel may be bent into the form of lines desired more easily than the profile steels of round or square cross-section because it has a flat

shape, and it has moreover the advantage as compared with the known cold-worked reinforcement steels which have been preferred because of their higher yield point values, that in it a high yield point for the purpose of attaining higher permissible steel stresses appears combined with the advantage of better adhesive strength. This adhesive strength makes it for example possible to dispense with the turning up of end hooks for the purpose of anchorage. It is likewise possible to dispense with an anchorage in the compression zone which is indispensable with all known profile steels, and tests have proved that the profile steel according to the invention need not extend beyond the end point according to calculation. A further particularly valuable advantage arises from the use of reinforcement steel according to the invention as a prestressed reinforcement in concrete constructions. This advantage consists in that owing to the repeated direct anchorage along the entire length of the reinforcement steel stresses are reliably transmitted between the concrete and the steel in contradistinction to the smooth drawn prestressed wires where such possibility of transmission does not exist, or as compared with the known reinforcements consisting of intertwined wires and spacers arranged between the same at places, where such a possibility of transmission exists to a small extent only. Accordingly the holder heads required with pre-stressed smooth wires can also be dispensed with.

Beside, at least the longitudinal rods may be subjected at one stage of the production process of the reinforcement steel according to the invention to an improving treatment increasing its strength properties, e.g., to a thermal treatment such as artificial ageing or "patenting." The same effect can alternatively be attained by the addition of appropriate strength-increasing alloy elements.

The new reinforcement steel is suitable for reinforced concrete structures of any kind.

We claim:

1. An integral reinforcing construction for reinforced concrete, which comprises two longitudinal rods of steel, each of a diameter ranging between 0.13 inch as a minimum and 1.2 inches as a maximum, and having a yield point exceeding 70,000 p.s.i. which extend parallel to each other, 0.8 to 1.2 inches apart, and transverse webs of softer steel interwelded at intervals to said longitudinal rods and extending at right angles to the longitudinal rods and having substantially flat side faces extending at right angles to the longitudinal rods and a width substantially equal to the diameter of the longitudinal rods, the ratio of the spacing between the transverse webs to the spacing between the longitudinal rods being less than

2.4

$\phi$

inches where  $\phi$  is the diameter of the longitudinal rods in inches.

2. A reinforcing construction as set forth in claim 1, in which the thickness of the webs is between 0.4  $\phi$  to 0.75  $\phi$ .

3. A reinforcing construction as set forth in claim 1, in which the longitudinal rods consist of cold-drawn steel.

4. A reinforcing construction as set forth in claim 1, in which the steel of the longitudinal rods has a relatively high content of alloying constituents selected of the class consisting of carbon and manganese and the steel of the transverse webs has a relatively low content of said alloying constituents.

5. An integral reinforcing construction for reinforced concrete, which comprises two longitudinal rods of steel, each of a diameter ranging between 0.13 inch as a minimum and 1.2 inches as a maximum, and having a yield point exceeding 70,000 p.s.i., which extend parallel to each other with a spacing of about 0.8 to 1.2 inches and

transverse webs of softer steel interwelded at intervals to said longitudinal rods and extending at right angles to the longitudinal rods and having substantially flat side faces extending at right angles to the longitudinal rods and having a width substantially equal to the diameter of the longitudinal rods, the ratio of the spacing between the transverse webs to the spacing between the longitudinal rods fulfilling the relation

$$10 \quad \frac{0.16 \cdot 10^{10}}{\phi f_s^2} \leq \frac{s}{a} \leq \frac{0.6 \cdot 10^{10}}{\phi f_s^2}$$

wherein  $f_s$  is the permissible steel stress in p.s.i.,  $\phi$  the diameter of the longitudinal rods,  $s$  is the spacing between the transverse webs and  $a$  is the spacing between said rods.

15 6. An integral reinforcing construction for reinforced concrete, which comprises two longitudinal rods of steel, each of a diameter ranging between 0.13 inch as a minimum and 1.2 inches as a maximum, and having a yield point exceeding 70,000 p.s.i. which extend parallel to each other about 0.8 to 1.2 inches apart and transverse webs of softer steel interwelded at intervals to said longitudinal rods and extending at right angles to the longitudinal rods and having flat side faces extending at right angles to the longitudinal rods and a width substantially equal to the diameter of the longitudinal rods, the ratio

$$\frac{s}{a}$$

30 of the spacing  $s$  of the transverse webs to the clearance  $a$  between the longitudinal rods fulfilling the relation

$$35 \quad \frac{0.32 \cdot 10^{10}}{\phi f_s^2} \leq \frac{s}{a} \leq \frac{1.2 \cdot 10^{10}}{\phi f_s^2}$$

wherein  $f_s$  is the permissible steel stress in p.s.i. and the diameter  $\phi$  of the longitudinal rods is  $\frac{1}{2}$  inch.

40 7. An integral reinforcing construction for reinforced concrete, which comprises two longitudinal rods of steel, each of a diameter ranging between 0.13 inch as a minimum and 1.2 inches as a maximum, and having a yield point exceeding 70,000 p.s.i. which extend parallel to each other with a spacing between them about equal to the diameter of said rods, and transverse webs of softer steel interwelded at intervals to said longitudinal rods and extending at right angles to the longitudinal rods and having substantially flat side faces extending at right angles to the longitudinal rods and a width substantially equal to the diameter of the longitudinal rods, the spacing of the transverse webs being less than about 8 inches.

45 8. A graded series of reinforcing elements for reinforced concrete, in which each element comprises two longitudinal rods of steel, each of a diameter ranging between 0.13 inch as a minimum and 1.2 inches as a maximum, and having a yield point exceeding 70,000 p.s.i., which extend parallel to each other with a spacing between them of about 0.8 to 1.2 inches and transverse webs of softer steel interwelded at intervals to said longitudinal rods and extending at right angles to the longitudinal rods and having flat side faces extending at right angles to the longitudinal rods and a width substantially equal to the diameter of the longitudinal rods, the element having the longitudinal rods largest in diameter fulfilling the relation

$$65 \quad \frac{1.3}{\phi} \leq \frac{s}{a} \leq \frac{2.4}{\phi}$$

70 76 wherein  $s$  is the spacing between said webs,  $a$  is the spacing between said rods, and  $\phi$  is the diameter of said rod in inches whereas in the elements having longitudinal rods smaller in diameter, the transverse webs have the same spacing as in the element having the longitudinal rods largest in diameter.

75 9. A graded series of reinforcing elements according to claim 8, characterized in the element having the longi-

11

tudinal rods largest in diameter the diameter of the longitudinal rods is  $\frac{1}{2}$  inch and the value

$$\frac{s}{a}$$

for all elements of the series fulfills the relation

$$2.6 \leq \frac{s}{a} \leq 4.8$$

the web spacing being the same in all elements of the 10 series.

12

References Cited in the file of this patent

UNITED STATES PATENTS

|   |           |            |               |
|---|-----------|------------|---------------|
| 5 | 468,841   | Stephenson | Feb. 16, 1892 |
|   | 1,096,685 | Cummings   | May 12, 1914  |
|   | 1,911,018 | Goeltz     | May 23, 1933  |
|   | 2,316,560 | Causey     | Apr. 13, 1943 |

FOREIGN PATENTS

|           |         |               |
|-----------|---------|---------------|
| France    | 594,184 | June 13, 1925 |
| Australia | 105,658 | Apr. 27, 1938 |